# EUROPEAN PATENT SPECIFICATION

(11) **EP 4 288 603 B1**
(45) Date of publication and mention of the grant of the patent: **08.07.2026**
(21) Application number: 22703919.5
(22) Date of filing: 02.02.2022
(51) Int. Cl.: D21H 17/16, D21H 17/37, D21H 17/62, D21H 17/67, D21H 17/68, D21H 21/16, D21H 21/18, D21H 23/14

(54) **PAPERMAKING METHOD**
PAPIERHERSTELLUNGSVERFAHREN
PROCÉDÉ DE FABRICATION DE PAPIER

(30) Priority: 02.02.2021 EP 21154736; 22.12.2021 EP 21217014
(43) Date of publication of application: 13.12.2023
(73) Proprietor: Billerud Aktiebolag (publ), 169 27 Solna (SE)
(72) Inventor: VALTANEN, Eero Antero, 33960 PIRKKALA (FI)
(74) Representative: Kransell & Wennborg KB
(86) International application number: PCT/EP2022/052384
(87) International publication number: WO 2022/167437

(56) References cited:
- EP-A1- 3 168 362
- WO-A1-2012/042115
- WO-A1-2015/075318
- WO-A1-2017/162920
- WO-A1-2018/229345
- WO-A1-2020/012074
- WO-A1-2020/128144

## Description

### TECHNICAL FIELD

The present disclosure relates to the field of papermaking.

### BACKGROUND

In the field of papermaking, it is difficult to achieve certain combinations of paper properties. As an example, it is generally challenging to produce a paper of high bending resistance that, at the same time, has smooth surfaces. This is because the calendering operation that is normally used to smoothen the surfaces also densifies the paper and thereby makes it floppy. Another example of conflicting properties are wet strength and recyclability since the latter requires repulping of the paper, which is typically hampered by the wet strength. Yet another example is that there is often a conflict between low porosity and good formation. This is because low porosity typically requires highly refined pulp that is often difficult to dewater. To overcome the dewatering problem, the headbox consistency may be increased and/or more retention chemicals may be added. Both these measures are however known impair formation.

WO 2020/128144 discloses a process for producing paper or board wherein an anionic polymer or cationic G-PAM may be added to the pulp.

WO 2018/229345 refers to a strength additive system for manufacturing of paper comprising cationic polymers with aldehyde functional groups and anionic copolymers obtained by polymerisation.

### SUMMARY

An objective of the present disclosure is to provide a method of producing a recyclable paper having relatively high wet strength. In some embodiments, it is also an objective that the paper exhibits at least one and preferably all of the following properties: good formation; low porosity; and low surface roughness without increasing the density too much.

Accordingly, there is provided a method of producing a paper on a paper machine, comprising the steps of:
a) providing a pulp;
b) adding cationic glyoxylated polyacrylamide (G-PAM) to the pulp, wherein the consistency of the pulp is in the range of 1.5-3.0 % when the cationic G-PAM is added;
c) forming a web from the pulp in a forming section comprising a head box;
d) pressing the web in a press section;
e) drying the web in a drying section; and
f) optionally calendering the web in a calender,
wherein the method further comprises adding an anionic polymer to the pulp before adding the cationic G-PAM.

In one embodiment the pulp is a mixture of hardwood pulp and softwood pulp.

In one embodiment the pulp is bleached.

In one embodiment the pulp is a kraft pulp, such as a mixture of a bleached hardwood pulp and a bleached softwood pulp.

In one embodiment the pulp is refined, e.g. such that the Schopper-Riegler number measured according to ISO 5267-1:1999 of the pulp in the head box is 20-30, preferably 22-30, such as 23-28. Said refining may comprise low consistency (LC) refining.

In one embodiment the pH of the pulp is in the range of 4.8-5.5 when the cationic G-PAM is added.

In one embodiment the pulp is not subjected to refining after the G-PAM addition.

In one embodiment cationic G-PAM is added in a total amount of 1.5-3.0 kg/tonne dry fibre, preferably 2.0-3.0 kg/tonne dry fibre, more preferably 2.5-3.0 kg/tonne dry fibre.

In one embodiment the anionic polymer is anionic polyacrylamide (A-PAM). The A-PAM may be added in a total amount of 0.20-1.00 kg/tonne dry fibre, preferably 0.25-0.75 kg/tonne dry fibre, more preferably 0.35-0.55 kg/tonne dry fibre.

In one embodiment the pH of the pulp is in the range of 6.5-8.0 when the anionic polymer is added.

In one embodiment the pulp is subjected to LC refining after the addition of the anionic polymer.

In one embodiment the method further comprises adding at least one hydrophobic size to the pulp.

The at least one hydrophobic size may comprise rosin size. Said rosin size may be added in a total amount of 1.0-4.0 kg/tonne dry fibre, preferably 1.5-3.0 kg/tonne dry fibre, more preferably 1.5-2.5 kg/tonne dry fibre.

The at least one hydrophobic size may comprise ASA or AKD, preferably AKD. Said AKD may be added in a total amount of 0.3-2.0 kg/tonne dry fibre, preferably 0.4-1.5 kg/tonne dry fibre, more preferably 0.4-1.0 kg/tonne dry fibre.

The pH of the pulp may be in the range of 4.8-5.5 when the at least one hydrophobic size is added.

The consistency of the pulp may be in the range of 1.5-3.0 % when the at least one hydrophobic size is added.

In one embodiment the pulp is not subjected to refining after the addition of the at least one hydrophobic size.

When the method comprises adding at least one hydrophobic size to the pulp it may further comprise adding alum to the pulp. Said alum may be added in a total amount of 2.0-8.5 kg/tonne dry fibre, preferably 2.5-5.5 kg/tonne dry fibre, more preferably 2.5-4.5 kg/tonne dry fibre.

In one embodiment said alum is added before said at least one hydrophobic size.

In one embodiment the consistency of the pulp in the head box is 0.20-0.60 %, preferably 0.30-0.55 %, more preferably 0.35-0.50 %.

In one embodiment the pH of the pulp in the head box is in the range of 4.8-5.5, preferably 5.0-5.5.

In one embodiment clay is added to the pulp, for example such an amount that the ash content of the paper is in the range of 2.0-5.5 %, such as 3.0-5.0 %. The point of addition of said clay may be in the short circulation.

In one embodiment, the method further comprises adding a dry strength agent to the pulp. The dry strength agent may be starch, preferably cationic starch. Said starch may be added in a total amount of 2.0-7.0 kg/tonne dry fibre, preferably 3.5-6.0 kg/tonne dry fibre.

In one embodiment the forming section comprises a wire shaker.

In one embodiment the cross directional dry content of the web is controlled by a steam box arranged at the downstream end of the forming section.

In one embodiment the press section comprises a shoe press. The shoe press may be operated at a line load of 650-950 kN/m, such as 750-900 kN/m. The press section may further comprise at least one press nip upstream the shoe press.

In one embodiment the calender is a soft nip calender. The line load of the soft nip calender may be in the range of 60-170 kN/m, preferably 80-140 kN/m, such as 100-140 kN/m. The hard roll of the soft nip calender may be heated, preferably to a temperature in the range of 100-200 °C, such as 120-180 °C.

In one embodiment the grammage measured according to ISO 536:2019 of the paper is at least 100 g/m².

In one embodiment the specific formation number measured according to SCAN-P 92:09 of the paper is below 1.00 √g/m, such as below 0.90 √g/m, such as below 0.85 √g/m.

In one embodiment the Bendtsen roughness measured according to SS-ISO 8791-2:2013 of at least one side of the paper is below 250 ml/min, preferably below 220 ml/min, more preferably below 160 ml/min.

In one embodiment the Bendtsen roughness measured according to SS-ISO 8791-2:2013 of both sides of the paper is below 600 ml/min, preferably below 500 ml/min, more preferably below 400 ml/min.

In one embodiment the Gurley value according to ISO 5636-5:2013 of the paper is above 50 s, preferably above 60 s, such as above 65 s.

In one embodiment the density measured according to ISO 534:2011 of the paper is 600-950 kg/m³, preferably below 600-920 kg/m³.

In one embodiment the wet tensile strength index measured according to ISO 1924-3:2005 in the machine direction (MD) of the paper is at least 8.0 Nm/g, preferably at least 9.5 Nm/g, more preferably above 11.0 Nm/g.

In one embodiment the wet tensile strength index measured according to ISO 1924-3:2005 in the cross direction (CD) of the paper is at least 5.5 Nm/g, preferably at least 6.5 Nm/g, more preferably at least 7.5 Nm/g.

In one embodiment the wet tensile stiffness index measured according to ISO 1924-3:2005 in the machine direction (MD) of the paper is at least 1000 Nm/g, preferably at least 1045 Nm/g, more preferably at least 1200 Nm/g.

In one embodiment the wet tensile stiffness index measured according to ISO 1924-3:2005 in the cross direction (CD) of the paper is at least 400 Nm/g, preferably at least 445 Nm/g, more preferably at least 545 Nm/g.

In one embodiment mixing of said cationic G-PAM with the pulp is aided by a pump. The pump may be arranged downstream the point of addition of said cationic G-PAM, but upstream a headbox pump. For example, the pump may be arranged upstream a wire pit, which in turn is arranged upstream the headbox pump.

In one embodiment the Cobb 60 s value measured according to ISO 535:2014 of at least one side of the paper is below 30 g/m², preferably below 25 g/m², more preferably below 23.5 g/m².

In one embodiment the Cobb 60 s value measured according to ISO 535:2014 of both sides of the paper is below 30 g/m², preferably below 25 g/m², more preferably below 23.5 g/m².

In one embodiment the method further comprises adding polyamino amide epichlorohydrin (PAE) resin to the pulp in a total amount of 0.15-1.75 kg/tonne dry fibre. The amount of PAE resin may be 0.25-1.50 kg/tonne dry fibre, preferably 0.30-1.25 kg/tonne dry fibre, such as 0.30-1.10 kg/tonne dry fibre or 0.40-1.25 kg/tonne dry fibre. The PAE may be added before the cationic G-PAM is added.

In one embodiment A-PAM is added to the pulp and the PAE resin is added after the A-PAM addition.

### DETAILED DESCRIPTION

There is thus provided a method of producing a paper on a paper machine, comprising the steps of:
a) providing a pulp;
b) adding cationic glyoxylated polyacrylamide (G-PAM) to the pulp, wherein the consistency of the pulp is in the range of 1.5-3.0 % when the cationic G-PAM is added;
c) forming a web from the pulp in a forming section comprising a head box;
d) pressing the web in a press section;
e) drying the web in a drying section; and
f) optionally calendering the web in a calender,
wherein the method further comprises adding an anionic polymer to the pulp before adding the cationic G-PAM.

In one embodiment, the pulp preferably a mixture of hardwood pulp and softwood pulp. This embodiment is particularly relevant for bleached pulp. The dry weight ratio of hardwood pulp to softwood pulp may be between 70:30 and 10:90, such as between 60:40 and 25:75, preferably between 60:40 and 30:70, more preferably between 55:45 and 40:60.

The pulp may be bleached or unbleached. When it is unbleached, it may be a 100% softwood pulp.

The pulp is preferably a kraft pulp. For example, it may be a mixture of a bleached hardwood sulphate pulp and a bleached softwood sulphate pulp.

Broke pulp is typically added, e.g. in a proportion of 5-30% (w/w). The broke pulp is preferably obtained from the same method. The broke pulp is typically added downstream a refining step. However, the broke pulp may be added upstream the addition of the anionic polymer (discussed below). In one embodiment, broke pulp is added downstream a refining step, but upstream of all additions of papermaking chemicals.

The method preferably comprises refining of the pulp, e.g. to such a degree that a Schopper-Riegler (SR) number of 20-30, preferably 22-30, such as 23-28. Refining can be carried out in different positions between the cook and the headbox. In any case, the SR number ranges given herein relate to the pulp in the head box. In the context of the present disclosure, SR numbers are measured according to ISO 5267-1:1999.

The refining normally comprises low consistency LC refining, e.g. refining at a consistency of 2-5 %, such as 3-4 %. In some embodiments comprising LC refining, no high consistency (HC) refining is carried out.

When the cationic G-PAM is added to the pulp, the pulp preferably has a pH in the range of 4.8-5.5, such as 5.0-5.5.

Preferably, refining is only carried out before the addition of the cationic G-PAM. Accordingly, in one embodiment of the method, the pulp is not subjected to any refining after the addition of the cationic G-PAM.

The total amount of cationic G-PAM added to the pulp may be 1.5-5.0 kg/tonne dry fibre, such as 1.5-3.0 kg/tonne dry fibre, preferably 2.0-3.0 kg/tonne dry fibre, such as 2.5-3.0 kg/tonne dry fibre.

As an example, the cationic G-PAM may be added to the pulp in the piping leading from the machine chest to the wire pit of the paper machine.

Mixing of said cationic G-PAM with the pulp may be aided by a pump. The pump is preferably arranged upstream a headbox pump (and, of course, downstream the point of addition of said cationic G-PAM). In one embodiment, the pump is arranged upstream a wire pit, which in turn is arranged upstream the headbox pump.

The method comprises adding an anionic polymer to the pulp, i.a. to balance the charge of the pulp. The anionic polymer may for example be anionic polyacrylamide (A-PAM). The total amount of A-PAM added to the pulp may be 0.20-1.00 kg/tonne dry fibre, preferably 0.25-0.75 kg/tonne dry fibre, more preferably 0.35-0.55 kg/tonne dry fibre. The anionic polymer is added to the pulp before the cationic G-PAM is added is added to the pulp. The pH of the pulp may be in the range of 6.5-8.0 when the anionic polymer is added. In one embodiment, LC refining is carried out before and after the addition of the anionic polymer. In such case, the amount of LC refining (measured as kWh/tonne dry fibre) may be higher before than after the addition of the anionic polymer.

The method may further comprise adding at least one hydrophobic size to the pulp, thereby reducing the water absorption of the paper and thus improving its durability in wet or humid conditions.

The at least one hydrophobic size preferably comprises rosin size. Rosin size may be added to the pulp in a total amount of 1.0-4.0 kg/tonne dry fibre, preferably 1.5-3.0 kg/tonne dry fibre, more preferably 1.5-2.5 kg/tonne dry fibre.

Further, the at least one hydrophobic size may comprise Alkenylsuccinic anhydride (ASA) or Alkylketene dimer (AKD), preferably AKD. AKD may be added to the pulp in a total amount of 0.3-2.0 kg/tonne dry fibre, preferably 0.4-1.5 kg/tonne dry fibre, more preferably 0.4-1.0 kg/tonne dry fibre.

Preferably, the at least one hydrophobic size comprises both rosin size and AKD.

When the at least one hydrophobic size is added, the pH of the pulp is preferably in the range of 4.8-5.5 and the consistency of the pulp is preferably in the range of 1.5-3.0 %.

In an embodiment, the pulp is not subjected to refining after the addition of the at least one hydrophobic size.

The at least one hydrophobic size is preferably added after the addition anionic polymer discussed above. As an example, the at least one hydrophobic size may be added to the pulp in the piping leading from the machine chest to the wire pit of the paper machine.

An embodiment of the method further comprises adding alum to the pulp, e.g. in a total amount of 2.0-8.5 kg/tonne dry fibre, preferably 2.5-5.5 kg/tonne dry fibre, more preferably 2.5-4.5 kg/tonne dry fibre. Alum is preferably added to the pulp before any hydrophobic size is added to the pulp.

In the method, the headbox consistency of the pulp may be 0.20-0.60 %, such as 0.30-0.55 %, such as 0.35-0.50 %, in particular when the grammage is above 100 g/m². The present inventors have managed to obtain good formation at this headbox consistency, also when the pulp is subjected to LC refining and papermaking chemicals are added.

To improve the formation, the forming section of the paper machine may comprise a wire shaker.

In an embodiment of the method, the cross directional dry content of the web is controlled by a steam box arranged at the downstream end of the forming section.

The pH of the pulp in the head box may be in the range of 4.8-5.5, preferably 5.0-5.5.

In an embodiment of the method, inorganic filler, such as clay, is added to the pulp. Inorganic filler may be added in such an amount that the ash content of the paper is in the range of 0.5-5.5 %, 2.0-5.5 %, such as 3.0-5.0 %. The addition of inorganic filler typically improves surface properties of the paper. A drawback of adding inorganic filler may however be lower strength properties. Also, addition of inorganic filler typically increases the density of the paper. Still, the present investors have managed to keep the density of the paper below 915 kg/m³ (in full scale trial 1 even below 890 kg/m³) while obtaining relatively high wet strength properties at an ash content of 4% (see table 1).

Clay is preferably added in the short circulation of the paper machine.

An embodiment of the method further comprises adding a dry strength agent to the pulp. The dry strength agent may be starch, preferably cationic starch. The total amount of starch that is added to the pulp may be 2.0-9.0 kg/tonne dry fibre, such as 2.0-7.0 kg/tonne dry fibre, preferably 3.5-6.0 kg/tonne dry fibre.

It has been found that to further improve the wet strength properties without significantly impairing recyclability, a relatively small amount (0.15-1.75 kg/tonne dry fibre) od PAE resin may be added to the pulp. A higher amount of PAE (i.e. 3 kg/tonne dry fibre) has been shown to reduce recyclability to an unacceptably low level.

The amount of PAE resin is preferably 0.25-1.50 kg/tonne dry fibre and more preferably 0.30-1.25 kg/tonne dry fibre, such as 0.30-1.10 kg/tonne dry fibre or 0.40-1.25 kg/tonne dry fibre.

The PAE resin is suitably added to the pulp before the cationic G-PAM is added. If A-PAM is added in the method, the PAE resin is preferably added to the pulp after the A-PAM addition.

The press section of the paper machine may comprise a shoe press, which may be operated at a line load of 650-950 kN/m, such as 750-900 kN/m. Upstream the shoe press, there may be at least one additional press nip, such as two additional press nips. The first of these may be operated at a line load of 40-90 kN/m, such as 50-70 kN/m, whereas the second may be operated at a line load of 50-100 kN/m, such as 60-90 kN/m. Hence the line load of the first press nip is preferably lower than the line load of the second press nip.

The calendering of step f) is carried out when low surface roughness is desired. The calender of step f) is preferably a soft nip calender, which may be operated at a line load of 60-170 kN/m, preferably 80-140 kN/m, such as 100-140 kN/m. The hard roll of the soft nip calender may be heated, preferably to a temperature in the range of 100-200 °C, such as 100-150 °C or 120-180 °C. The moisture content of the web may be 7.0-8.5 % when entering the calender of step f).

The method of the present disclosure facilitates the production of a paper having certain properties:

The grammage of the paper is typically 50-200 g/m², such as 70-160 g/m². The method of the present disclosure is particularly beneficial in case of a grammage of at least 100 g/m², such as at least 120 g/m². The papers produced in the full-scale trials 1-3 described below all had a grammage above 120 g/m² (see table 1). According to the present disclosure, grammage is measured according to ISO:536:2019.

The Bendtsen roughness of at least one side of the paper is preferably below 250 ml/min, preferably below 220 ml/min, more preferably below 160 ml/min. In one embodiment, the Bendtsen roughness of both sides of the paper is below 600 ml/min, such as below 500 ml/min, such as below 400 ml/min. In the context of the present disclosure, Bendtsen roughness is measured according to SS-ISO 8791-2:2013. To obtain low Bendtsen roughness values, step f) is carried out.

The density (measured according to ISO 534:2011) of the paper is preferably below 950 kg/m³, more preferably below 920 kg/m³. At the same time, the density is normally above 600 kg/m³, more preferably below 650 kg/m³. The present method is not intended for tissue paper or similar lightweight paper.

As shown in table 1 below, a paper having a Bendtsen roughness of below 160 ml/min on the printing side and below 400 ml/min on the reverse side as well as a density below 920 kg/m² was produced in full scale trial 2.

In some embodiments, the specific formation number of the paper is preferably below 1.00 √g/m, such as below 0.90 √g/m, such as below 0.85 √g/m.The specific formation number is measured according to SCAN-P 92:09, preferably using an Ambertec Beta Formation Tester

In some embodiments, the Gurley value (measured according to ISO 5636-5:2013) is preferably above 50 s, more preferably above 60 s, such as above 65 s. A typical upper limit may be 150 s or 100 s. Higher Gurley values are obtained by a relatively high degree of refining, in particular LC refining, and/or calendering.

As shown in table 1 below, the papers produced in full scale trials 1-3 had specific formation numbers below 0.85 √g/m and Gurley values above 65 s.

Preferably, the wet tensile strength index in the machine direction (MD) of the paper is at least 8.0 Nm/g, more preferably at least 9.5 Nm/g, such as above 11.0 Nm/g. In the cross direction (CD), the wet tensile strength index of the paper is preferably at least 5.5 Nm/g, more preferably at least 6.5 Nm/g, such as at least 7.5 Nm/g. Wet tensile strength index is sometimes referred to as only "wet tensile index". Wet tensile strength index is measured according to the standard ISO 1924-3:2005, which specifies a wetting time of 10 min.

Preferably, the wet tensile stiffness index in the machine direction (MD) of the paper is at least 1000 Nm/g, more preferably at least 1045 Nm/g, such as at least 1200 Nm/g. In the cross direction (CD), the wet tensile stiffness index of the paper is preferably at least 400 Nm/g, more preferably at least 445 Nm/g, such as at least 545 Nm/g. Wet tensile stiffness index is measured according to the standard ISO 1924-3:2005, which specifies a wetting time of 10 min.

As shown in table 1 below, a paper having a wet tensile strength index above 11.0 Nm/g in MD and above 7.5 Nm/g in CD as well as a wet tensile stiffness index above 1200 Nm/g in MD and above 545 Nm/g in CD was produced in full scale trial 1. This paper was also recyclable.

To improve performance in wet/humid conditions, it is also preferred that the Cobb 60 s value of at least one side of the paper is below 30 g/m², preferably below 25 g/m², more preferably below 23.5 g/m². In one embodiment, the Cobb 60 s value of both sides of the paper is below 30 g/m², such as below 25 g/m², such as below 23.5 g/m². The Cobb 60 s value is measured according to ISO 535:2014.

### EXAMPLES

### Full scale trial 1

A pulp mixture was prepared by mixing never-dried bleached softwood kraft pulp and never-dried bleached hardwood kraft pulp in a 50:50 dry weight ratio. The pH of the pulp mixture was adjusted to about 7 and the pulp mixture was then subjected to low consistency (LC) refining (130 kWh/tonne dry fibre, consistency = about 4%). Broke pulp was added to the LC-refined pulp mixture and the resulting pulp was subjected to thick stock screening. The proportion of broke pulp was about 15% (w/w). A-PAM (Fennobond 85E) was then added to the pulp in an amount of about 0.5 kg/tonne dry fibre. After the addition of A-PAM, the pulp was subjected to post LC refining (21 kWh/tonne dry fibre, consistency = about 3.3%).

The post LC-refined pulp was routed to the machine chest, in which alum was dosed in an amount of 3-4 kg/tonne dry fibre such that the pH of the pulp was adjusted to about 5.2. Dyes (violet and blue) and cationic starch (Raisamyl 50021, 5 kg/tonne dry fibre) were also added to the pulp in the machine chest. Rosin size (2.5 kg/tonne dry fibre), AKD (0.8 kg/tonne dry fibre) and cationic G-PAM (Fennobond 3150E, 2.8 kg/tonne dry fibre) were added to the pulp in the piping leading from the machine chest to the wire pit. The consistency of the pulp in this position was 2.2%. After the additions of rosin size, AKD and cationic G-PAM, but before the wire pit, the pulp was subjected to pumping.

Between the wire pit and the headbox pump, "heavier" particles (like sand and metal) were separated from the pulp by means of a hydrocyclones system. Air was removed from the pulp by a Perivac deaerator. Downstream the headbox pump, but upstream the headbox, cationic retention aid (Fennopol K 7526P, 0.15 kg/tonne dry fibre) and anionic retention aid/silica (FennoSil 5000, 0.45 kg/tonne dry fibre) were added. The cationic retention aid was added before machine screens and the silica was added after the machine screens. Kaolin clay was added to the short circulation in such an amount that the ash content of the final paper was about 4%.

In the headbox, the pH of the pulp was still about 5.2. The SR number of the pulp was 24-28. The headbox consistency of the pulp was about 0.45%. A paper web was formed in a forming section comprising a one-ply fourdrinier wire and a wire shaker. At the downstream end of the forming section, the web was steamed by means of a steam box to obtain an even moisture profile in the cross direction before the press section.

The press section had three nips: first a single-felted nip operated at a line load of 60 kN/, then another single-felted nip operated at a line load of 70 kN/m and finally a shoe press nip operated at a line load of 850 kN/m. The web from the press section was dried in a drying section. After the drying section, at a moisture of 7.5-8.0 %, the web was subjected to soft nip calendering at a line load of 103 kN/m. The hard roll of the soft nip calender was heated to 150 °C. The properties of the resulting paper are presented in table 1 below.

A paper corresponding to that produced in full scale trial 1, but having a basis weight of 120 g/m², was tested according to PTS-method PTS-RH:021/97 (Draft Oct 2019) 'Identification of the recyclability of paper and board packages and of graphic print products' - Category II: Paper and board for Recycling (PfR) that are predominantly used in the manufacture of packaging papers. The paper passed all the tests of the method and was thus found to be "Recyclable" (despite the wet strength properties).

### Full scale trial 2

Full scale trail 2 was carried out in the same way as full scale trial 1 with the following exceptions:
- The hardwood pulp was a resuspended marked pulp instead of a never-dried pulp;
- The energy consumption in the first LC refining was 112 kWh/tonne dry fibre instead of 130 kWh/tonne dry fibre;
- The energy consumption in the post LC refining was 19 kWh/tonne dry fibre instead of 21 kWh/tonne dry fibre;
- The amount of cationic retention aid was 0.20 kg/tonne dry fibre instead of 0.15 kg/tonne dry fibre; and
- The line load of soft nip calender was 130 kN/m instead of 103 kN/m.

The properties of the paper produced in trial 2 are presented in table 1 below.

### Full scale trial 3

Full scale trail 3 was carried out in the same way as full scale trial 1 with the following exceptions:
- The energy consumption in the first LC refining was 80 kWh/tonne dry fibre instead of 130 kWh/tonne dry fibre;
- The energy consumption in the post LC refining was 20 kWh/tonne dry fibre instead of 21 kWh/tonne dry fibre;
- The line load of soft nip calender was 120 kN/m instead of 103 kN/m; and
- The hard roll of the soft nip calender was heated to 130 °C instead of 150 °C.

The properties of the paper produced in trial 3 are presented in table 1 below.

**Table 1. Properties of the papers produced in full scale trials 1-3. PS means printing side. RS means reverse side. MD means machine direction. CD means cross direction. The formation number and the specific formation number were measured using an Ambertec Beta Formation Tester according to the standard SCAN-P 92:09.**

| **Full scale trial #** | **1** | **2** | **3** |
|---|---|---|---|
| Grammage (g/m²) | 137.7 | 138.4 | 139 |
| Thickness (µm) | 155 | 153 | 152 |
| Density (kg/m³) | 888 | 905 | 9¹4 |
| Gurley (s) | 76 | 71 | 83 |
| Bendtsen Roughness PS (ml/min) | 217 | 139 | 213 |
| Bendtsen Roughness RS (ml/min) | 436 | 348 | 456 |
| Cobb PS (g/m²) | 20 | 20 | 19.7 |
| Cobb RS (g/m²) | 21 | 21 | 20.7 |
| Formation number (g/m²) | 9.8 | 9.7 | 8.8 |
| Specific Formation number (√g/m) | 0.83 | 0.82 | 0.75 |
| Tensile Strength MD (kN/m) | 11.6 | 11.5 | 12.52 |
| Tensile Strength CD (kN/m) | 7.1 | 7.1 | 7.87 |
| Tensile Strain at break MD (%) | 2.2 | 2.1 | 2.73 |
| Tensile Strain at break CD (%) | 7 | 6.5 | 7.2 |
| Tensile Stiffness MD (kN/m) | 1323 | 1274 | 1273 |
| Tensile Stiffness CD (kN/m) | 634 | 627 | 652 |
| Wet Tensile Strength MD, 10 min (kN/m) | 1.63 | N/A | 1.91 |
| Wet Tensile index MD, 10 min (Nm/g) | 11.84 | N/A | 13.74 |
| Wet Tensile Strength CD, 10 min (kN/m) | 1.12 | N/A | 1.21 |
| Wet Tensile index CD, 10 min (Nm/g) | 8.13 | N/A | 8.71 |
| Wet Tensile Stiffness MD, 10 min (kN/m) | 174 | N/A | N/A |
| Wet Tensile Stiffness index MD, 10 min (Nm/g) | 1264 | N/A | N/A |
| Wet Tensile Stiffness CD, 10 min (kN/m) | 77 | N/A | N/A |
| Wet Tensile Stiffness index CD, 10 min (Nm/g) | 559 | N/A | N/A |
| Wet Tensile Strength MD, 15 min (kN/m) | 1.55 | 1.46 | 1.72 |
| Wet Tensile Index MD, 15 min (Nm/g) | 11.26 | 10.55 | 12.37 |
| Wet Tensile Strength CD, 15 min (kN/m) | 1.0 | 0.94 | 1.1 |
| Wet Tensile Index CD, 15 min (Nm/g) | 7.26 | 6.79 | 7.91 |
| Wet Tensile Stiffness MD, 15 min (kN/m) | 164 | 170 | 136 |
| Wet Tensile Stiffness index MD, 15 min (Nm/g) | 1191 | 1228 | 978 |
| Wet Tensile Stiffness CD, 15 min (kN/m) | 62 | 71 | 50 |
| Wet Tensile Stiffness index CD, 15 min (Nm/g) | 450 | 513 | 360 |

Table 1 shows that recyclable papers having relatively high wet strength properties were successfully produced in trial 1-3. In addition, the produced papers exhibited satisfactory specific formation numbers, low porosity (i.e. high Gurley values) and low surface roughness (in particular on the printing side (PS)), while the density was kept at an acceptable level.

That beneficial formation numbers were obtained despite the additions of various papermaking chemicals is, at least in part, attributable to the order in which the papermaking chemicals were added as well as their concentrations and the pH and/or consistency of the pulp at their points of addition.

### Full scale trial 4

A never-dried bleached softwood kraft pulp was provided. The pH of the pulp was adjusted to about 7.5 and the pulp was then subjected to high consistency (HC) refining (about 170 kWh/tonne dry fibre, consistency about 32%) followed by low consistency (LC) refining (36 kWh/tonne dry fibre, consistency = about 4%). Broke pulp was added to the refined pulp and the resulting pulp was subjected to thick stock screening. The proportion of broke pulp was about 15% (w/w). A-PAM (Fennobond 85E) was then added to the pulp in an amount of about 0.4 kg/tonne dry fibre. After the addition of A-PAM, the pulp was subjected to post LC refining (about 16 kWh/tonne dry fibre, consistency = about 3.3%).

The post LC-refined pulp was routed to the machine chest, in which alum was dosed in an amount of 3-4 kg/tonne dry fibre such that the pH of the pulp was adjusted to about 5.2. Dyes (violet and blue) and cationic starch (Raisamyl 50021, about 3.5 kg/tonne dry fibre) were also added to the pulp in the machine chest. Rosin size (about 2 kg/tonne dry fibre), AKD (0.5 kg/tonne dry fibre) and cationic G-PAM (Fennobond 3150E, 2.5 kg/tonne dry fibre) were added to the pulp in the piping leading from the machine chest to the wire pit. The consistency of the pulp in this position was 2.2%. After the additions of rosin size, AKD and cationic G-PAM, but before the wire pit, the pulp was subjected to pumping.

Between the wire pit and the headbox pump, "heavier" particles (like sand and metal) were separated from the pulp by means of a hydrocyclones system. Air was removed from the pulp by a Perivac deaerator. Downstream the headbox pump, but upstream the headbox, cationic retention aid (Fennopol K 7526P, 0.15 kg/tonne dry fibre) and anionic retention aid/silica (FennoSil 5000, 0.3 kg/tonne dry fibre) were added. The cationic retention aid was added before machine screens and the silica was added after the machine screens.

In the headbox, the pH of the pulp was still about 5.2. The SR number of the pulp was 23. The headbox consistency of the pulp was about 0.2%. A paper web was formed in a forming section comprising a one-ply fourdrinier wire and a wire shaker. At the downstream end of the forming section, the web was steamed by means of a steam box to obtain an even moisture profile in the cross direction before the press section.

The press section had three nips; first a single-felted nip operated at a line load of 60 kN/, then another single-felted nip operated at a line load of 70 kN/m and finally a shoe press nip operated at a line load of 850 kN/m.

The web from the press section was dried in a drying section having seven dryer groups and a Clupak unit (used to compact/microcrêpe the web) arranged in series. The Clupak unit was arranged between dryer groups four and three, which means that the paper web was dried in the drying section both before and after the Clupak unit. No calendering was carried out.

The resulting paper was tested according to PTS-method PTS-RH:021/97 (Draft Oct 2019) 'Identification of the recyclability of paper and board packages and of graphic print products' - Category II: Paper and board for Recycling (PfR) that are predominantly used in the manufacture of packaging papers. The paper passed all the tests of the method and was thus found to be "Recyclable" (despite the wet strength properties). Other properties of the paper are presented in table 2 below.

### Full scale trial 5

A never-dried unbleached softwood kraft pulp was provided. The pH of the pulp was adjusted to about 8 and the pulp was then subjected to high consistency (HC) refining (about 160 kWh/tonne dry fibre, consistency about 32%) followed by low consistency (LC) refining (85 kWh/tonne dry fibre, consistency = about 4%). Broke pulp was added to the refined pulp and the resulting pulp was subjected to thick stock screening. The proportion of broke pulp was about 15% (w/w). A-PAM (Fennobond 85E) was then added to the pulp in an amount of about 0.4 kg/tonne dry fibre. After the addition of A-PAM, the pulp was subjected to post LC refining (about 27 kWh/tonne dry fibre, consistency = about 3.3%).

The post LC-refined pulp was routed to the machine chest, in which alum was dosed in an amount of 7 kg/tonne dry fibre such that the pH of the pulp was adjusted to about 5.3. Cationic starch (Raisamyl 50021, 5 kg/tonne dry fibre) was also added to the pulp in the machine chest. Rosin size (about 1.5 kg/tonne dry fibre), AKD (0.4 kg/tonne dry fibre) and cationic G-PAM (Fennobond 3150E, 2.8 kg/tonne dry fibre) were added to the pulp in the piping leading from the machine chest to the wire pit. The consistency of the pulp in this position was 2.2%. After the additions of rosin size, AKD and cationic G-PAM, but before the wire pit, the pulp was subjected to pumping.

Between the wire pit and the headbox pump, larger pieces were separated from the pulp by means of a hydrocyclones system. Air was removed from the pulp by a Perivac deaerator. Downstream the headbox pump, but upstream the headbox, cationic retention aid (Fennopol K 7526P, 0.2 kg/tonne dry fibre) and anionic retention aid/silica (FennoSil 5000, 0.2 kg/tonne dry fibre) were added. The cationic retention aid was added before machine screens and the silica was added after the machine screens.

In the headbox, the pH of the pulp was still about 5.3. The SR number of the pulp was 20. The headbox consistency of the pulp was about 0.2%. A paper web was formed in a forming section comprising a one-ply fourdrinier wire and a wire shaker. At the downstream end of the forming section, the web was steamed by means of a steam box to obtain an even moisture profile in the cross direction before the press section.

The press section had three nips; first a single-felted nip operated at a line load of 60 kN/, then another single-felted nip operated at a line load of 70 kN/m and finally a shoe press nip operated at a line load of 850 kN/m.

The web from the press section was dried in a drying section having seven dryer groups and a Clupak unit (used to compact/microcrêpe the web) arranged in series. The Clupak unit was arranged between dryer groups four and three, which means that the paper web was dried in the drying section both before and after the Clupak unit. No calendering was carried out.

The properties of the paper produced in trial 5 are presented in table 2 below. Further, the inventors expect the paper produced in trial 5 to be recyclable according to the PTS method discussed above.

**Table 2. Properties of the papers produced in full scale trials 4 and 5. PS means printing side. RS means reverse side. MD means machine direction. CD means cross direction.**

| **Full scale trial #** | **4** | **5** |
|---|---|---|
| Grammage (g/m²) | 75.7 | 72.3 |
| Gurley (s) | 17.3 | 19.1 |
| Bendtsen Roughness PS (ml/min) | 635 | 786 |
| Bendtsen Roughness RS (ml/min) | 1133 | 1197 |
| Cobb (g/m²) | 21.1 | 23.3 |
| Brightness (%) | 83.5 | N/A |
| Tensile Strength MD (kN/m) | 6.1 | 7.48 |
| Tensile Strength CD (kN/m) | 4.6 | 4.56 |
| Tensile index MD (Nm/g) | 80.8 | 103.4 |
| Tensile index CD (Nm/g) | 60.3 | 63.3 |
| Tensile Strain at break MD (%) | 6.5 | 6.8 |
| Tensile Strain at break CD (%) | 8.7 | 8.4 |
| Tear strength MD (mN) | 1039 | 884 |
| Tear strength CD (mN) | 1125 | 1081 |
| Tear index MD (mNm²/g) | 13.7 | 12.1 |
| Tear index CD (mNm²/g) | 14.8 | 14.8 |
| Wet Tensile Strength MD, 10 min (kN/m) | 0.81 | 1.05 |
| Wet Tensile index MD, 10 min (Nm/g) | 10.7 | 14.5 |
| Burst strength (kPa) | 517 | 579 |
| Burst index (kPam²/g) | 6.8 | 8.1 |

### Full scale trial 6

A pulp mixture was prepared by mixing never-dried bleached softwood kraft pulp and never-dried bleached hardwood kraft pulp in a 70:30 dry weight ratio. The pH of the pulp mixture was adjusted to about 7 and the pulp mixture was then subjected to low consistency (LC) refining (80 kWh/tonne dry fibre, consistency = about 4%). Broke pulp was added to the LC-refined pulp mixture and the resulting pulp was subjected to thick stock screening. The proportion of broke pulp was about 15% (w/w). A-PAM (Fennobond 85E) was then added to the pulp in an amount of 0.4 kg/tonne dry fibre. After the addition of A-PAM, the pulp was subjected to post LC refining (15 kWh/tonne dry fibre, consistency = about 3.3%).

The post LC-refined pulp was routed to the machine chest, in which alum was dosed in an amount of 3-4 kg/tonne dry fibre such that the pH of the pulp was adjusted to about 5.2. Dyes (violet and blue) and cationic starch (Raisamyl 50021, 5 kg/tonne dry fibre) were also added to the pulp in the machine chest. Rosin size (2.2 kg/tonne dry fibre), AKD (0.7 kg/tonne dry fibre) and cationic G-PAM (Fennobond 3150E, 2.8 kg/tonne dry fibre) were added to the pulp in the piping leading from the machine chest to the wire pit. The consistency of the pulp in this position was 2.2%. After the additions of rosin size, AKD and cationic G-PAM, but before the wire pit, the pulp was subjected to pumping.

Between the wire pit and the headbox pump, "heavier" particles (like sand and metal) were separated from the pulp by means of a hydrocyclones system. Air was removed from the pulp by a Perivac deaerator. Downstream the headbox pump, but upstream the headbox, cationic retention aid (Fennopol K 7526P, 0.15 kg/tonne dry fibre) and anionic retention aid/silica (FennoSil 5000, 0.45 kg/tonne dry fibre) were added. The cationic retention aid was added before machine screens and the silica was added after the machine screens. Kaolin clay was added to the short circulation in such an amount that the ash content of the final paper was about 2%.

In the headbox, the pH of the pulp was still about 5.2. The SR number of the pulp was 24-28. The headbox consistency of the pulp was about 0.35%. A paper web was formed in a forming section comprising a one-ply fourdrinier wire and a wire shaker. At the downstream end of the forming section, the web was steamed by means of a steam box to obtain an even moisture profile in the cross direction before the press section.

The press section had three nips: first a single-felted nip operated at a line load of 60 kN/, then another single-felted nip operated at a line load of 70 kN/m and finally a shoe press nip operated at a line load of 850 kN/m. The web from the press section was dried in a drying section. After the drying section, at a moisture of 7.0-7.5 %, the web was subjected to soft nip calendering at a line load of 150 kN/m. The hard roll of the soft nip calender was heated to 130°C. Properties of the resulting paper are presented in table 3 below.

### Full scale trial 7

Full scale trail 7 was carried out in the same way as full scale trial 6 with the following exceptions:
- 1 kg/tonne PAE resin (Kymene GHP20 from Solenis) was added to the pulp in the machine chest;
- The amount of A-PAM was 0.6 kg/tonne dry fibre instead of 0.4 kg/tonne dry fibre;
- The amount of cationic starch was 7 kg/tonne dry fibre instead of 5 kg/tonne dry fibre;
- Kaolin clay was added to the short circulation in such an amount that the ash content of the final paper was 1% instead of 2%.

Properties of the paper produced in trial 7 are presented in table 3 below.

### Full scale trial 8

Full scale trail 8 was carried out in the same way as full scale trial 7 with the following exceptions:
- The amount of cationic G-PAM was 4.0 kg/tonne dry fibre instead of 2.8 kg/tonne dry fibre; and
- The amount of A-PAM was 0.8 kg/tonne dry fibre instead of 0.6 kg/tonne dry fibre.

Properties of the paper produced in trial 8 are presented in table 3 below.

**Table 3. Properties of the papers produced in full scale trials 6-8. PS means printing side. RS means reverse side. MD means machine direction. CD means cross direction.**

| **Full scale trial #** | | | **6** | **7** | **8** |
|---|---|---|---|---|---|
| Grammage (g/m²) | | | 137.7 | 137.9 | 138.7 |
| Thickness (µm) | | | 149 | 148 | 151 |
| Density (kg/m³) | | | 923 | 929 | 916 |
| Gurley (s) | | | 86.5 | 105.5 | 89 |
| Bendtsen Roughness PS (ml/min) | | | 221 | 207 | 219 |
| Bendtsen Roughness RS (ml/min) | | | 392 | 385 | 388 |
| Cobb PS (g/m²) | | | 19.8 | 19.9 | 19.9 |
| Cobb RS (g/m²) | | | 20.5 | 20.8 | 20.0 |
| Formation number (g/m²) | | | 10.4 | 9.4 | N/A |
| Specific Formation number (√g/m) | | | 0.89 | 0.80 | N/A |
| Tensile Strength MD (kN/m) | | | 14.0 | 14.9 | 14.7 |
| Tensile Strength CD (kN/m) | | | 7.5 | 8.0 | 7.9 |
| Tensile Strain at break MD (%) | | | 2.3 | 2.5 | 2.4 |
| Tensile Strain at break CD (%) | | | 7.6 | 8.0 | 7.8 |
| Tensile Stiffness MD (kN/m) | | | 1344 | 1379 | 1341 |
| Tensile Stiffness CD (kN/m) | | | 587 | 608 | 613 |
| Wet Tensile Strength MD, 15 min (kN/m) | | | 1.8 | 2.1 | 2.4 |
| Wet Tensile Index MD, 15 min (Nm/g) | | | 13.2 | 14.9 | 17.2 |
| Wet Tensile Strength CD, 15 min (kN/m) | | | 1.0 | 1.1 | 1.3 |
| Wet Tensile Index CD, 15 min (Nm/g) | | | 7.0 | 8.2 | 9.2 |
| Wet Tensile Stiffness MD, 15 min (kN/m) | | | 206 | 196 | 204 |
| Wet Tensile Stiffness index MD, 15 min (Nm/g) | | | 1492 | 1421 | 1471 |
| Wet Tensile Stiffness CD, 15 min (kN/m) | | | 55 | 62 | 65 |
| Wet Tensile Stiffness index CD, 15 min (Nm/g) | | | 396 | 445 | 469 |
| Recyclability (PTS-RH 021/97) | Disintegratability | Total reject | 0.14% | 0.23% | 1.87% |
| | | Recyclability | 99.86% | 99.77% | 98.13% |
| | Sheet formation | Adhesive impurities | None | None | None |
| | | Optical inhomogenities | None | None | None |
| Overall recyclability rating | | | Recyclable | Recyclable | Recyclable |

Table 3 shows that high wet strength properties can be increased further by adding PAE and more cationic G-PAM without significantly reducing recyclability.

## Claims

1. A method of producing a paper on a paper machine, comprising the steps of:
a) providing a pulp, such as a mixture of hardwood pulp and softwood pulp;
b) adding cationic glyoxylated polyacrylamide (G-PAM) to the pulp, wherein the consistency of the pulp is in the range of 1.5-3.0 % when the cationic G-PAM is added;
c) forming a web from the pulp in a forming section comprising a head box;
d) pressing the web in a press section;
e) drying the web in a drying section; and
f) optionally calendering the web in a calender,
wherein the method further comprises adding an anionic polymer to the pulp before adding the cationic G-PAM.

2. The method of claim 1, wherein the pulp is refined, e.g. such that the Schopper-Riegler number measured according to ISO 5267-1:1999 of the pulp in the head box is 20-30, preferably 22-30, such as 23-28.

3. The method of claim 1 or 2, wherein the pH of the pulp is in the range of 4.8-5.5 when the cationic G-PAM is added.

4. The method of any one of the preceding claims, wherein cationic G-PAM is added in a total amount of 1.5-3.0 kg/tonne dry fibre, preferably 2.0-3.0 kg/tonne dry fibre, more preferably 2.5-3.0 kg/tonne dry fibre.

5. The method of any one of the preceding claims, wherein the pulp is not subjected to refining after the cationic G-PAM addition.

6. The method of any one of the preceding claims, wherein the anionic polymer is anionic polyacrylamide (A-PAM).

7. The method of claim 6, wherein the pH of the pulp is in the range of 6.5-8.0 when the anionic polymer is added.

8. The method of any one of the preceding claims, further comprising adding at least one hydrophobic size, such as rosin size and/or AKD, to the pulp.

9. The method of claim 8, wherein the pH of the pulp is in the range of 4.8-5.5 and the consistency of the pulp is in the range of 1.5-3.0 % when the at least one hydrophobic size is added.

10. The method of any one of the preceding claims, further comprising adding clay to the pulp in such an amount that the ash content of the paper is in the range of 2.0-5.5 %, such as 3.0-5.0 %.

11. The method of any one of the preceding claims, wherein consistency of the pulp in the head box is 0.20-0.60 %, preferably 0.30-0.55 %, more preferably 0.35-0.50 %.

12. The method of any one of the preceding claims, wherein the calender is a soft nip calender operated at a line load of 60-170 kN/m, such as 80-140 kN/m, such as 100-140 kN/m, and/or a temperature of 100-200 °C, such as 100-150 °C or 120-180 °C.

13. The method of any one of the preceding claims, wherein the grammage measured according to ISO 536:2019 of the paper is at least 100 g/m² and/or the density measured according to ISO 534:2011 of the paper is at least 600 kg/m³.

14. The method of any one of the preceding claims, wherein the specific formation number measured according to SCAN-P 92:09 of the paper is below 1.00 √g/m, such as below 0.90 √g/m, such as below 0.85 √g/m.

## Patentansprüche

1. Verfahren zur Herstellung eines Papiers auf einer Papiermaschine, umfassend die Schritte:
a) Bereitstellen einer Pulpe, beispielsweise einer Mischung aus Hartholzzellstoff und Weichholzzellstoff;
b) Zugeben von kationischem glyoxyliertem Polyacrylamid (G-PAM) zu der Pulpe, wobei die Konsistenz der Pulpe im Bereich von 1,5 bis 3,0 % liegt, wenn das kationische G-PAM zugegeben wird;
c) Bilden einer Papierbahn aus der Pulpe in einem Formierabschnitt, der einen Stoffauflauf aufweist;
d) Pressen der Papierbahn in einem Pressenabschnitt;
e) Trocknen der Papierbahn in einem Trockenabschnitt; und
f) optionales Kalandrieren der Papierbahn in einem Kalander,
wobei das Verfahren ferner das Zugeben eines anionischen Polymers zu dem Faserstoff vor dem Zugeben des kationischen G-PAM umfasst.

2. Verfahren nach Anspruch 1, wobei die Pulpe raffiniert wird, beispielsweise derart, dass die nach ISO 5267-1:1999 gemessene Schopper-Riegler-Zahl der Pulpe im Stoffauflauf 20 bis 30, vorzugsweise 22 bis 30, beispielsweise 23 bis 28 beträgt.

3. Verfahren nach Anspruch 1 oder 2, wobei der pH-Wert der Pulpe im Bereich von 4,8 bis 5,5 liegt, wenn das kationische G-PAM zugegeben wird.

4. Verfahren nach einem der vorhergehenden Ansprüche, wobei das kationische G-PAM in einer Gesamtmenge von 1,5 bis 3,0 kg/Tonne Trockenfaser, vorzugsweise 2,0 bis 3,0 kg/Tonne Trockenfaser, stärker bevorzugt 2,5 bis 3,0 kg/Tonne Trockenfaser zugegeben wird.

5. Verfahren nach einem der vorhergehenden Ansprüche, wobei die Pulpe nach der Zugabe des kationischen G-PAM keiner Raffination unterzogen wird.

6. Verfahren nach einem der vorhergehenden Ansprüche, wobei das anionische Polymer anionisches Polyacrylamid (A-PAM) ist.

7. Verfahren nach Anspruch 6, wobei der pH-Wert der Pulpe im Bereich von 6,5 bis 8,0 liegt, wenn das anionische Polymer zugegeben wird.

8. Verfahren nach einem der vorhergehenden Ansprüche, ferner umfassend das Zugeben mindestens einer hydrophoben Leimung, beispielsweise Harzleimung und/oder AKD, zu der Pulpe.

9. Verfahren nach Anspruch 8, wobei der pH-Wert der Pulpe im Bereich von 4,8 bis 5,5 liegt und die Konsistenz der Pulpe im Bereich von 1,5 bis 3,0 % liegt, wenn die mindestens eine hydrophobe Leimung zugegeben wird.

10. Verfahren nach einem der vorhergehenden Ansprüche, ferner umfassend das Zugeben von Ton zu der Pulpe in einer solchen Menge, dass der Aschegehalt des Papiers im Bereich von 2,0 bis 5,5 %, beispielsweise 3,0 bis 5,0 %, liegt.

11. Verfahren nach einem der vorhergehenden Ansprüche, wobei die Konsistenz der Pulpe im Stoffauflauf 0,20 bis 0,60 %, vorzugsweise 0,30 bis 0,55 %, stärker bevorzugt 0,35 bis 0,50 %, beträgt.

12. Verfahren nach einem der vorhergehenden Ansprüche, wobei der Kalander ein Softnip-Kalander ist, der mit einer Linienlast von 60 bis 170 kN/m, beispielsweise 80 bis 140 kN/m, beispielsweise 100 bis 140 kN/m, und/oder bei einer Temperatur von 100 bis 200 °C, beispielsweise 100 bis 150 °C oder 120 bis 180 °C, betrieben wird.

13. Verfahren nach einem der vorhergehenden Ansprüche, wobei die nach ISO 536:2019 gemessene Grammatur des Papiers mindestens 100 g/m² beträgt und/oder die nach ISO 534:2011 gemessene Dichte des Papiers mindestens 800 kg/m³ beträgt.

14. Verfahren nach einem der vorhergehenden Ansprüche, wobei die nach SCAN-P 92:09 gemessene spezifische Formationszahl des Papiers unter 1,00 √g/m, beispielsweise unter 0,90 √g/m, beispielsweise unter 0,85 √g/m, liegt.

## Revendications

1. Procédé de fabrication d'un papier sur une machine à papier, comprenant les étapes suivantes :
a) la fourniture d'une pâte à papier, telle qu'un mélange de pâte de bois dur et de pâte de bois tendre ;
b) l'ajout de polyacrylamide glyoxylé cationique (G-PAM) à la pâte à papier, dans lequel la consistance de la pâte à papier se situe dans la plage comprise entre 1,5 et 3,0 % lors de l'ajout du G-PAM cationique ;
c) la formation d'une nappe à partir de la pâte dans une section de formation comprenant une caisse de tête ;
d) le pressage de la nappe dans une section de pressage ;
e) le séchage de la nappe dans une section de séchage ; et
f) le calandrage facultatif de la nappe dans une calandre,
dans lequel le procédé comprend en outre l'ajout d'un polymère anionique à la pâte avant l'ajout du G-PAM cationique.

2. Procédé selon la revendication 1, dans lequel la pâte est raffinée, par exemple de telle sorte que l'indice de Schopper-Riegler, mesuré selon la norme ISO 5267-1:1999, de la pâte dans la caisse de tête soit compris entre 20 et 30, de préférence compris entre 22 et 30, tel que compris entre 23 et 28.

3. Procédé selon la revendication 1 ou la revendication 2, dans lequel le pH de la pâte se situe dans la plage comprise entre 4,8 et 5,5 lorsque le G-PAM cationique est ajouté.

4. Procédé selon l'une quelconque des revendications précédentes, dans lequel le G-PAM cationique est ajouté en une quantité totale comprise entre 1,5 et 3,0 kg/tonne de fibres sèches, de préférence comprise entre 2,0 et 3,0 kg/tonne de fibres sèches, et plus préférablement comprise entre 2,5 et 3,0 kg/tonne de fibres sèches.

5. Procédé selon l'une quelconque des revendications précédentes, dans lequel la pâte n'est pas soumise à un raffinage après l'ajout du G-PAM cationique.

6. Procédé selon l'une quelconque des revendications précédentes, dans lequel le polymère anionique est du polyacrylamide anionique (A-PAM).

7. Procédé selon la revendication 6, dans lequel le pH de la pâte se situe dans la plage comprise entre 6,5 et 8,0 lorsque le polymère anionique est ajouté.

8. Procédé selon l'une quelconque des revendications précédentes, comprenant en outre l'ajout d'au moins un agent d'encollage hydrophobe, tel qu'un agent d'encollage à base de colophane et/ou de l'AKD, à la pâte.

9. Procédé selon la revendication 8, dans lequel le pH de la pâte est compris entre 4,8 et 5,5 et la consistance de la pâte est comprise entre 1,5 et 3,0 % lorsque ledit au moins un agent d'encollage hydrophobe est ajouté.

10. Procédé selon l'une quelconque des revendications précédentes, comprenant en outre l'ajout d'argile à la pâte en une quantité telle que la teneur en cendres du papier se situe dans la plage comprise entre 2,0 et 5,5 %, telle que comprise entre 3,0 et 5,0 %.

11. Procédé selon l'une quelconque des revendications précédentes, dans lequel la consistance de la pâte dans la caisse de tête est comprise entre 0,20 et 0,60 %, de préférence comprise entre 0,30 et 0,55 %, et plus préférablement comprise entre 0,35 et 0,50 %.

12. Procédé selon l'une quelconque des revendications précédentes, dans lequel la calandre est une calandre à pincement souple fonctionnant à une charge linéaire comprise entre 60 et 170 kN/m, telle que comprise entre 80 et 140 kN/m, telle que comprise entre 100 et 140 kN/m, et/ou à une température comprise entre 100 et 200 °C, telle que comprise entre 100 et 150 °C ou comprise entre 120 et 180 °C.

13. Procédé selon l'une quelconque des revendications précédentes, dans lequel le grammage du papier, mesuré selon la norme ISO 536:2019, est d'au moins 100 g/m² et/ou la densité du papier, mesurée selon la norme ISO 534:2011, est d'au moins 600 kg/m³.

14. Procédé selon l'une quelconque des revendications précédentes, dans lequel l'indice de formation spécifique du papier, mesuré selon la norme SCAN-P 92:09, est inférieur à 1,00 vg/m, tel qu'inférieur à 0,90 vg/m, tel qu'inférieur à 0,85 vg/m.
